

## UNITED STATES PATENT OFFICE

2,426,277

## METHOD OF MAKING A WATER AND OIL THINNABLE COATING COMPOSITION

Gustavus Harry Miller, Portland, Oreg.

No Drawing. Application April 18, 1944,  
Serial No. 531,658

7 Claims. (Cl. 106—227)

1

The present invention relates to surface coating compositions such as varnishes, paints and the like, more particularly to those of the type which may be thinned with water, and to methods for making the same.

Protective coating compositions usually comprise a vehicle consisting of a base of a drying oil or a resin, or a mixture thereof, dissolved in a volatile thinner with or without a quantity of pigment, and also a small amount of a drier. Following application, the thinner evaporates, leaving the base material, which upon drying forms the protective film. A large proportion of the total cost of the usual coating composition is represented by the thinner constituent which is added primarily merely to facilitate the application or spreading of the composition over a surface. Thinners, such as turpentine, coal tar or petroleum fractions and the like, are relatively costly and considerable research has been directed toward the reduction of the quantity required of this particular component.

Attempts have been made heretofore to employ water in resin or oil base vehicles, but, on the whole, the results have been only mediocre due to the inherently water insoluble nature of the vehicle base materials. Various compositions have been developed in which a limited quantity of water is introduced into the product in the manufacturing process in the form of a water-in-oil emulsion. The amount of water which it has been possible heretofore to add into the vehicle has been relatively small, generally less than half of the usual amount of solvent thinner. Additional amounts of water cannot subsequently be added, as by the user, for further thinning such compositions, and any attempt so to do has an opposite effect, that is of increasing the viscosity rather than decreasing it. In such compositions the water component is merely a diluent and not a true thinner. In order to thin such varnishes or paints for application it is necessary to employ a spirit thinner as in the case of the more conventional varnishes or paints. It is desirable to provide coating compositions such as varnishes, paints, or the like, which may readily be thinned as required with water and which, at the same time, are fast drying, leaving protective films which are water resistant, abrasion resistant, and having a surface which is either flat, semi-flat, semi-glossy, or glossy, depending upon the selection of the vehicle base materials.

It is a general object of the present invention, therefore, to provide a new and improved surface coating composition which may be thinned with water.

It is a further object to provide a new and improved surface coating composition having a resinous or drying oil vehicle base which may be thinned with water and, upon application to a

2

surface, dries rapidly to form a protective film which can be made to possess desired qualities as to water and abrasion resistance or surface smoothness, depending upon variations in the vehicle base components.

More specifically, it is an object of the invention to provide a surface coating composition comprising a protective film forming material which is insoluble in water and having admixed therewith a quantity of a dispersant which, when dissolved with such material by a small amount of a common solvent, forms a product which may be thinned with water.

A further specific object of the invention is to provide a new and improved dispersant which is particularly suitable for adding to a vehicle base such as a resin, drying oil, or other water insoluble film forming substance, to produce a coating composition which may readily be thinned with water.

And another object is to provide a new and improved dispersion medium which may be combined with a common oil paint base and form a coating composition therewith which may be thinned either with conventional spirit thinners, or with water as desired.

In the preparation of surface coating compositions according to the present invention, I employ a dispersion medium, or dispersant, which is compatible with ordinary vehicle solvents and also with water, and capable of forming a clear, stable dispersion therebetween. Thus a small amount of the dispersant is first mixed with a selected vehicle base material and dissolved therewith by a suitable common solvent in an amount sufficient to provide a clear solution. Since the dispersant is also water soluble, water may then be added to reduce the viscosity of the solution as may be required for application to a surface.

The dispersant itself is comprised essentially of an alkali metal resinate prepared by reacting an aqueous mixture of abietic acid, or rosin, and a relatively strong alkali base such as sodium hydroxide or potassium hydroxide. As will be more fully explained hereinafter, the dispersant may be prepared according to numerous modifications depending upon the particular type of coating composition under consideration. It may also be produced in different forms for use under various specific conditions.

The resinate dispersant is freely soluble in such ordinary vehicle solvents as aliphatic alcohols, turpentine, toluol, benzol, petroleum naphthas, and aromatic petroleum fractions of the solvent type, as well as in water. The dispersant may be mixed with such resinous film forming materials as rosin, natural resins, and dispersable synthetic resins comprising those of the coumarone-indene, phenolic, maleic or alkyd types, and if not readily soluble therein can be dissolved there-

with by a small amount of a suitable solvent which is common to both such as turpentine, toluol, benzol, aromatic petroleum solvents, or petroleum thinners. The dispersant may also be added to and dissolved in any of the typical drying oils such as linseed oil, soy bean oil, and similar vegetable oils, also refined fish oils, and whale oil. The viscosity of the resultant solution may be adjusted with the addition of a small amount of a suitable common solvent. The term "common solvent" as used in the specification and in the claims denotes substances having properties that will dissolve both the dispersant and the vehicle base material, such as resins or oils or mixtures thereof, into clear solutions.

The resins and oils may be combined in any desired proportions in accordance with the particular properties as desired in the final coating film with or without the addition of such other ingredients as pine oil, drying oil, fatty acids, or a small amount of a solution of a cellulose ester, such as ethyl cellulose, or a solution of chlorinated rubber for improving the brushing, flexibility, and abrasion characteristics of the coating and for retarding the drying sufficiently for facilitating the application thereof to surfaces, or for improving water resistance of the film. This vehicle, which may be pigmented or not, as desired, is miscible with water in all proportions and which may be added thereto for thinning purposes and, if unpigmented, may be applied to surfaces either as a clear varnish or a clear wall sealer, depending upon the extent of thinning. No special precautions need be taken in adding the water as a thinner other than mere stirring of the mixture while slowly adding the water until the desired consistency has been reached. The dispersion or suspension thus formed is exceedingly stable, that is, the composition may be allowed to stand over relatively long periods of time without any noticeable separation of water taking place. The alkali metal resinate dispersant which is employed is a low cost material as compared with the cost of the usual emulsifiers or binders, and, due to the fact that the use of the dispersant eliminates the need for solvent as a thinner and enables the use of water for such purpose, a very substantial saving is effected in the total cost of the ingredients required to produce a given quantity of surface coating composition ready for application.

The vehicle may be packaged as a thick, viscous liquid leaving to the consumer the matter of thinning for application, and since water is the only thinner required, a very definite advantage results to the consumer, not only from the standpoint of cost, but also as to the ready availability of the thinner.

Another advantage of coating compositions according to one modification of the present invention resides in the fact that the vehicle may be packaged in a concentrated form containing no water, and consequently, the composition will not freeze at temperatures higher than the freezing temperatures for the various oils or solvents employed. Because only a minimum amount of solvent is present, the fire hazard of the composition is greatly minimized. When employed with long oil, medium oil, and short oil varnishes, the dispersant materially improves the adhesion and drying properties without detrimentally clouding or raising the viscosity of such varnishes.

Following the spreading of the vehicle, the volatile solvent and the water will evaporate in turn from the layer of the substance. The resultant

film will level out smoothly and evenly without the formation of bubbles or droplets of water, leaving the dried film free from pits or pin holes which has characterized many of the water emulsion type oil paints developed heretofore. Since the vehicle base materials are not miscible with water, the resultant film becomes water insoluble upon drying. While the resinate dispersant remains in the film and, even though it was initially water soluble, this property is lost in the dried film due to the fact that each minute particle thereof is thoroughly surrounded and bonded by the principal water insoluble vehicle ingredients.

Pigments as used in the paint industry, such as titanium dioxide, the various lithopones, lead, zinc, and synthetic iron oxides or the like, and suitable coloring matter as desired may be added to the dispersant containing vehicle and produced and packaged in the form of a thick paste, leaving to the consumer, again, the matter of thinning with water to the desired consistency for spreading. It will be obvious, of course, that the water may be added before packaging, if desired in the case of ready-mixed type paints.

As will be pointed out more fully hereinafter, the dispersant may be mixed in the dry powdered form with such dry varnish and paint film forming materials as powdered resins and the like and combined with dry pigments, which mixture can conveniently be shipped in paper bags. The specified amount of common solvent may be added by the consumer to the mixture to first form a paste and which may then be thinned with water in suitable proportions to prepare the composition for application to surfaces.

In order that the invention may more fully be understood and practiced by those skilled in the art to which it pertains, the following formulas and examples are given:

#### DISPERSANT A

|                             | Parts by weight |
|-----------------------------|-----------------|
| Abietic acid                | 16              |
| Potassium hydroxide         | 3               |
| Borax                       | 1               |
| Water (distilled preferred) | 44              |

The abietic acid is first pulverized and then mixed with sixteen parts of water in a beaker large enough to hold twice the volume of the total ingredients. The potassium hydroxide, borax and four parts of water are added to another beaker and stirred until dissolved and, while still hot from the heat of reaction between alkali and water, are added to the first mixture with constant stirring until the mass is thoroughly mixed. Heat is then applied and the remaining twenty-four parts of water are slowly stirred into the combined mixtures. When the temperature reaches 85°-90° C. the mass begins to boil and becomes liquid with foam on the top. After boiling for about a minute or two, with continuous stirring, the heat is removed and the mass allowed to cool to room temperature and then stirred again until smooth. The resultant product, light amber in color and of a thin paste-like consistency, is a potassium-borate-abietic acid resinate with approximately a thirty-one per cent solids content and which may be used in this form as a dispersant in the manner described.

Sodium hydroxide may be substituted for potassium hydroxide and either plain, hydrogenated or polymerized gum or wood rosin for abietic acid in the above formula, and since sodium hydroxide and rosin are relatively lower in cost, the use of these materials may be desired for reasons of

greater economy. If sodium hydroxide and rosin are used in the preparation of the dispersant following the same procedure as outlined above, it will be observed that the resultant product will separate into two distinct phases. One of the components will be a light straw-colored, foamy mass, while the other component will be a relatively dark colored liquid. Both of these components are effective as dispersants and may be used separately or in a combined form. If a dispersant in a dry powder form is desired, then the foamy mass may be dried, as by spray drying, and used in this form. Because of its light color, the vehicle compounded therewith will be correspondingly light in color. On the other hand the liquid phase, being relatively dark in color, will correspondingly darken the vehicle compounded therewith. If a vehicle base is to be prepared and in which a relatively small percentage of water is not objectionable, the light colored, foamy mass may be used in the wet form without first drying it.

For general use, as in coating compounds which are not to be subjected to subfreezing temperatures and which, hence, may contain a certain amount of water, the two separate phases of the last mentioned dispersant may be recombined into a clear liquid dispersant with the addition thereto of a small amount of a common solvent. For such a solvent I prefer to use one to three parts toluol, benzol, petroleum aromatic solvent, mineral spirits or a mixture thereof, to one part of a relatively high boiling point alcohol, such as butyl alcohol. The addition of butyl alcohol imparts certain desirable properties to the dispersant in that it enhances the solubility characteristics of the common solvent. Butyl alcohol, a polar liquid, is a good wetting agent, miscible with water, and lowers the viscosity of both the dispersant and paint vehicle to which it is added. Since it also lowers the freezing point of water thinnable paints, it assists in their application to cold, damp and frosty surfaces as in the case of camouflage coatings or other exterior paints.

The amount of water may be reduced very materially from that stated above to lower the moisture content of the dispersant. For example, by reducing the water to twelve parts a dispersant of a soft, paste-like consistency is produced which has a solids content of approximately sixty-two per cent.

The following is an example of a dispersant which may be prepared in a single vessel and in one operation.

#### DISPERSANT B

| Parts by weight                                                          |    |  |
|--------------------------------------------------------------------------|----|--|
| Petroleum thinner (No. 9 Union Oil Company of California, or equivalent) | 4  |  |
| No. 40 aromatic petroleum solvent (Union Oil Company of California)      | 1  |  |
| W. W. rosin                                                              | 16 |  |
| Sodium hydroxide                                                         | 2  |  |
| Borax                                                                    | 2  |  |
| Water (distilled preferred)                                              | 8  |  |

The petroleum thinner, aromatic solvent, rosin, sodium hydroxide and borax are added in the order stated to a beaker equal in size to twice the volume of the total ingredients and thoroughly mixed. Eight parts of water are slowly added with constant stirring to form a soft straw color paste which after cooling over night separates into a liquid and a granular solid. The liquid is decanted and the remaining semi-stiff paste of a

pale straw color is a dispersant soluble in all ordinary liquid vehicle components.

If it is desired to prepare the dispersant in a dry form, as for storage and future use, the following modification is recommended.

#### DISPERSANT C

|                                                                        | Parts by weight |
|------------------------------------------------------------------------|-----------------|
| Hydrogenated rosin (Staybelite, Hercules Power Company, or equivalent) | 16              |
| Pine oil                                                               | 1               |
| Potassium hydroxide                                                    | 3               |
| Borax                                                                  | 1               |
| Water (distilled preferred)                                            | 8               |

15. The previously pulverized rosin and one part pine oil, are thoroughly mixed in a beaker large enough to hold twice the volume of the total ingredients. The sodium hydroxide and borax are dissolved in eight parts water and the solution is immediately added to the rosin mixture and stirred less than a minute. The liquid will separate from the polymerized rosin and with the aid of a spatula, it is squeezed out and decanted. It is only necessary to have the hydrogenated rosin come in contact with the alkali solution for a very short time, not over a minute. Heat is applied and the mixture is cooked at a temperature of about 85° to 90° C. until the last trace of water has been evaporated after which it is poured into a cooling pan to harden. Although the solid dispersant requires breaking up by the user, it is more compact than a powdered or pulverized product, requires less shipping space and is not as susceptible to oxidation or combustion and therefore no antioxidant is required. This solid dispersant may be considered as a commercially dry product. Further modifications of dispersants which may be prepared in a solid form will be described later.
20. Hydrogenated rosin is used in this formula because of its inherent resistance to oxidation and stability to heat and sunlight. It is also pointed out that this type of rosin has certain apparent advantages over abietic acid and standard grades of rosin due to its non-yellowing properties when used in the formulation of white interior and exterior paints. The small amount of pine oil is used in this case to prevent excessive foaming during the reaction.
25. The proportions as set forth in the above formulas as well as in those following are not to be taken as being critical in that they are susceptible of considerable variation. For example, to every sixteen parts of abietic acid or rosin, the relative quantity of potassium or sodium hydroxide may, in general, be varied from one to four parts with satisfactory results, while the borax may be varied successfully from one-half to two and one-half parts. It is to be understood that even these ranges are not to be taken as definite, though the results obtained are in general less satisfactory as these ranges are exceeded.

30. The borax functions in the manner of a buffer and prevents excessive darkening of the resinate. While such darkening does not materially affect the quality of the products as a dispersant, the dark color is generally undesirable, particularly if clear, pale, or light colored varnishes or mixing and grinding vehicles are to be produced. On the other hand, the larger the amount of borax employed, the weaker will be the dispersing value for a given quantity of the product. Instead of borax, any other suitable buffer may be used, such as either monosodium, disodium or tri-
- 35.
- 40.
- 45.
- 50.

- 55.
- 60.
- 65.
- 70.
- 75.

sodium phosphate, or trisodium pyrophosphate. In one example of a dispersant given later no borax or other buffer is used so this is not an essential ingredient.

The following example illustrates the use of the dispersant in one of its simpler forms, as described above, in a common, interior, oil base paint.

## EXAMPLE 1

## Pigment

|                                                | Parts by weight |
|------------------------------------------------|-----------------|
| Titanium dioxide (water dispersable preferred) | 250             |
| Lithopone H. O. (water dispersable preferred)  | 125             |
| Zinc oxide XX                                  | 40              |
| Talc                                           | 150             |
| Asbestine                                      | 75              |

## Vehicle

|                                                                                      | Parts by weight |
|--------------------------------------------------------------------------------------|-----------------|
| Limed rosin, China-wood oil, varnish 30 gal. long, 40% solids, acid No. 8 to 12      | 180             |
| Gloss oil, 60% solids (N-Glo-5-Y, General Naval Stores Company, Inc., or equivalent) | 40              |
| Aromatic petroleum solvent (No. 40, Union Oil Company of California, or equivalent)  | 90              |

The varnish, gloss oil, petroleum solvent and pigment ingredients are added to a heavy duty mixer in the order and amounts as stated above with constant stirring and thoroughly mixed. This mixture is then transferred to a conventional paint mill and ground forming one of the usually accepted interior white semi-flat wall paste paints and which does not thin with water. However, it can readily be made capable of being thinned with water by adding to it a small quantity of dispersant as given below. It will be obvious that the dispersant will dissolve readily in the above paste paint due to the common solvent contained in the vehicle.

|                         | Parts by weight |
|-------------------------|-----------------|
| Dispersant (62% solids) | 30              |
| Above paste             | 90              |

The resultant paint paste can be thinned to brush consistency with thirty parts by weight of water.

This semi-flat interior paint, also used as an enamel undercoat, is of a short liquid type that brushes easily, levels and hides well, flows out smoothly and after drying over night, provides a hard tough film that may be washed repeatedly with cold water.

It is pointed out, that even though the dispersant is added to the above oil vehicle paint to make it water thinnable, it may still be thinned with the usual spirit thinners. Thus if it is to be applied to new wood then water should not be used because of its tendency to raise the grain and spirit thinners should be used instead for the first coat. For subsequent coats, or over old paint, or on new surfaces other than wood, the same paint may be used thinned with water.

## EXAMPLE 2

The outside paint of the following example, instead of using varnish, gloss oil and petroleum aromatic solvent as the vehicle, uses linseed oil as the sole vehicle binder for the pigment so that a more flexible paint film is provided which will

dry to a semi-gloss finish within a period of twenty-four hours.

## Pigment

|                                    | Parts by weight |
|------------------------------------|-----------------|
| Titanium dioxide (70% barium base) | 40              |
| Titanium dioxide                   | 96              |
| Zinc oxide XX                      | 16              |
| Asbestine                          | 6               |
| 10 Talc                            | 6               |

## Vehicle

|                                         | Parts by weight |
|-----------------------------------------|-----------------|
| Boiled linseed oil (pale preferred)     | 45              |
| Pale kettle bodied linseed oil (body Q) | 4               |

The vehicle is placed in a mixer and the pigments in the order and amounts as stated above are slowly added to the vehicle with constant stirring and thoroughly mixed. This mixture is then transferred to a conventional paint mill and ground and the resultant product, which cannot be thinned with water, is one of the usually accepted outside white paste paints though also recommended as an undercoat in two coat paint systems.

## Paste paint

|                               | Parts by weight |
|-------------------------------|-----------------|
| The above outside white paste | 90              |
| 30 Dispersant (62% solids)    | 27              |

Linseed oil fatty acids (double distilled preferred) 2 These ingredients are thoroughly mixed together to provide a water thinnable paste paint. To reduce the paste to brush consistency, twenty-seven parts of water are added. The resultant semi-gloss paint brushes easily, levels and hides well, and after drying twenty-four hours, provides a tough film that may be washed repeatedly with cold water.

The dispersants may be modified considerably from the simple forms given above so as to provide improved characteristics to the final coating material. The following example is illustrative of numerous possible modifications particularly suitable for use with outside paints.

## DISPERSANT D

|                                                                                     | Parts by weight |
|-------------------------------------------------------------------------------------|-----------------|
| 50 Polymerized rosin (poly pale resin, Hercules Powder Company, or equivalent)      | 32              |
| Aromatic petroleum solvent (No. 40, Union Oil Company of California, or equivalent) | 7               |
| 55 Butyl alcohol (normal preferred)                                                 | 7               |
| Sodium hydroxide                                                                    | 6               |
| Borax                                                                               | 2               |
| Water (distilled preferred)                                                         | 13              |
| Boiled linseed oil (pale preferred)                                                 | 15              |

60 The previously pulverized polymerized rosin, aromatic petroleum solvent, butyl alcohol, sodium hydroxide and borax are added to a beaker large enough to hold at least twice the volume of the total ingredients, and thoroughly mixed. Water is then slowly added with constant stirring and the heat of reaction between sodium hydroxide and water facilitates solution of all the ingredients. Fifteen parts linseed oil is promptly added to the hot solution and stirring is continued to produce a smooth soft paste having a vehicle solids content of approximately sixty-seven per cent and a water content of fifteen per cent. The linseed oil is added to improve the flow and gloss of the final paint product as will be 75 more fully described in the following example.

Butyl alcohol enhances the solubility characteristics of the ingredients and together with the aromatic petroleum is an excellent solvent for the resin. The butyl alcohol in the dispersant also contributes to the essential compatibility of the various liquids in the final product.

The product of Dispersant D is substantially more than merely a dispersant and is in the nature of a combination dispersant and vehicle. It may be thinned as it is with water and used as a varnish or clear wall sealer, or pigment may be added with a small amount of solvent to form a paste paint which may then be thinned with water and used for coating interior surfaces. It is particularly suitable, however, for use in the preparation of a heavily pigmented outside paint as will next be described.

#### EXAMPLE 3

##### Pigment

| Parts by weight                                         |     |  |
|---------------------------------------------------------|-----|--|
| White lead paste (lead carbonate ground in linseed oil) | 200 |  |
| Titanium dioxide                                        | 140 |  |
| Zinc oxide XX                                           | 80  |  |
| Asbestine                                               | 30  |  |
| Talc                                                    | 30  |  |

##### Vehicle

| Parts by weight                                                                     |     |  |
|-------------------------------------------------------------------------------------|-----|--|
| Ester gum, China-wood oil, varnish 30 gal. long, 40% solids, acid No. 8 to 12       | 31  |  |
| Pale kettle bodied linseed oil (body Q)                                             | 16  |  |
| Boiled linseed oil (pale preferred)                                                 | 105 |  |
| Aromatic petroleum solvent (No. 40, Union Oil Company of California, or equivalent) | 8   |  |
| Gum turpentine                                                                      | 1   |  |

The liquids are added to a standard heavy duty mixer and the lead paste and pigments in their order and amounts as stated above are slowly added to the vehicle with constant stirring and thoroughly mixed. This mixture is then transferred to a conventional paint mill and ground and the resultant product is one of the usually accepted durable outside white paste paints and which cannot be thinned with water. However, this paint can be made so as to be thinnable with water by combining a dispersant therewith as follows:

| Parts by weight       |    |  |
|-----------------------|----|--|
| Dispersant D          | 5  |  |
| The above paste paint | 25 |  |

The product of formula D, an alkali metal resinate, not only forms an excellent dispersant but also acts as a drier for the paint much like other resinate driers used in drying paint films. Because it is a combined oil and resin drier instead of a linoleate drier, it contributes to the formation of a harder, tougher paint film. No additional drier is needed unless a quicker dust free film is desired, then a small amount of cobalt naphthanate or resinate may be added as a top drier. The paint brushes easily, levels well, hides nicely, is white and dries to a smooth semi-gloss finish over night after which it may be readily washed with cold water. A higher gloss finish is produced by the application of a second coat.

In the preparation of a high gloss paint, as will next be described, pale kettle bodied linseed oil, commonly used as an enamel liquid, is employed instead of boiled linseed oil. Butyl alcohol is used for the same reasons as above.

#### DISPERSANT E

| Parts by weight |                                                                                 |    |
|-----------------|---------------------------------------------------------------------------------|----|
| 5               | Polymerized rosin (poly pale resin, Hercules Powder Company, or equivalent)     | 32 |
|                 | Potassium hydroxide                                                             | 8  |
|                 | Petroleum paint thinner (No. 9, Union Oil Company of California, or equivalent) | 7  |
| 10              | Butyl alcohol (normal preferred)                                                | 7  |
|                 | Water (distilled preferred)                                                     | 10 |
|                 | Pale kettle bodied linseed oil (body Q)                                         | 8  |

The rosin, potassium hydroxide, paint thinner and butyl alcohol are mixed together and the water is slowly added with constant stirring, while the heat of reaction between alkali and water completes the dissolution of the polymerized rosin. The linseed oil is then added to the resultant soft paste and thoroughly mixed therewith to provide a heavy bodied liquid dispersant. 20 It will be noted that no borax is employed in this instance.

#### EXAMPLE 4

##### Vehicle

| Parts by weight |                                                                                      |    |
|-----------------|--------------------------------------------------------------------------------------|----|
| 25              | Dispersant E                                                                         | 4  |
|                 | Gloss oil, 60% solids (N-Glo-5-Y, General Naval Stores Company, Inc., or equivalent) | 10 |

The above ingredients are thoroughly mixed and a clear, straw-color water thinnable paint vehicle is formed thereby.

##### Paste paint

| Parts by weight |                                              |    |
|-----------------|----------------------------------------------|----|
| 35              | Titanium oxide (water dispersable preferred) | 30 |
|                 | Above paint vehicle                          | 30 |

These ingredients are thoroughly mixed together to provide a water thinnable interior gloss paste paint, two volumes of which may be thinned with one volume of water for brushing consistency. The resultant paint brushes easily, hides very nicely, flows and covers well and dries to a smooth glossy film that is unusually white and which can readily be washed with cold water drying over night.

Linseed oil fatty acids are used in the succeeding example to lower the pH value, to release surface tension and also provide slip, for easier brush application, while pine oil is added to assist the flow and leveling properties. Sodium hydroxide is used in place of potassium hydroxide to lower the cost of the final product.

#### DISPERSANT F

| Parts by weight |                                                                                 |    |
|-----------------|---------------------------------------------------------------------------------|----|
| 55              | Polymerized rosin (poly pale resin, Hercules Powder Company, or equivalent)     | 16 |
|                 | Pine oil (double distilled preferred)                                           | 4  |
|                 | Sodium hydroxide                                                                | 3  |
| 60              | Borax                                                                           | 1  |
|                 | Water (distilled preferred)                                                     | 8  |
|                 | Petroleum paint thinner (No. 9, Union Oil Company of California, or equivalent) | 16 |
| 65              | Boiled linseed oil (pale refined preferred)                                     | 16 |
|                 | Linseed oil fatty acids (double distilled preferred)                            | 3  |

The rosin and one part pine oil are first thoroughly mixed in a beaker. The sodium hydroxide and borax are dissolved in eight parts water and the resultant solution while still hot from the heat of reaction is immediately added to the rosin mixture and stirred less than a minute. The liquid will separate from the polymerized 75 rosin and with the aid of a spatula, can be

## 11

squeezed out and decanted. The alkali treated rosin is then heated to approximately 90° C. whereupon it becomes fluid and the heat is then removed. The petroleum paint thinner and boiled linseed oil are promptly added in their order to the hot liquid resin, followed with three parts of pine oil and three parts linseed oil fatty acids and thoroughly mixed together. The resultant product free from water is a liquid dispersant.

## EXAMPLE 5

## Vehicle

## Parts by weight

Dispersant F-----30

Alkyd resin solution (50% solids in mineral spirits—No. 1323 Aroplaz, Stroock & Wittenerberg, or equivalent)-----25

## Paste paint

## Parts by weight

Titanated lithopone (Tidolith 44K, United Color & Pigment Company, or equivalent)-----40

Above vehicle-----20

This is a water thinnable paste paint and which can be reduced with fifteen parts by weight of water for brush consistency. The resultant paint brushes easily, levels well, hides very nicely, is white and dries to a smooth semi-gloss film over night and can then be readily washed with cold water.

In the preparation of a dry dispersant for storage and distribution in such form, vehicle resins may be combined therewith so as to simplify the compounding of the paint by the ultimate consumer. Maleic resin is combined with the dispersant in the following formula.

## DISPERSANT G

## Parts by weight

Polymerized rosin (poly pale resin, Hercules Powder Company, or equivalent)-----16

Sodium hydroxide-----3

Borax-----1

Water (distilled preferred)-----8

Pine oil (double distilled preferred)-----1

Boiled linseed oil (pale preferred)-----1

Maleic resin (No. 520 Arochem, Stroock & Wittenerberg, or equivalent)-----48

The previously pulverized polymerized rosin, a sodium hydroxide and borax are added to a beaker large enough to hold twice the volume of the total ingredients, the water is added and the materials are stirred with a glass rod until thoroughly mixed. Nearly eight parts of water will separate from the solid materials and which is decanted. The mixture is then cooked at a temperature of about 85° to 90° C. for three to five minutes, or until dissolved. The pine oil and linseed oil are then added and cooking is continued at a temperature sufficient to bring the materials to the boiling point, whereupon forty-eight parts maleic resin, which has been simultaneously heated to 250° to 260° C. in a separate container, are immediately added and the combined materials are then cooked until a drop on glass becomes clear and brittle at room temperature. The resultant mass is then poured into a cooling pan to harden forming a clear hard combined dispersant and resin. This material may be shipped or stored until it is to be used when it may be dissolved in an equal amount by weight of aromatic petroleum solvent, toluol, turpentine or the like, or a mixture thereof and ten to fifteen per cent by weight butyl alcohol, forming

## 12

a solution which is a clear liquid which can be used as it is a paint vehicle, varnish or clear sealer, that will thin with water in all proportions.

## EXAMPLE 6

Formula G, made with polymerized rosin in combination with a maleic resin having a melting point of 145° C. may also be used as in the following example to provide a dried film which will be highly resistant to abrasion, while the alkyd resin solution, as part of the completed vehicle, is necessary to increase the water resistance of the final product.

## Vehicle

## Parts by weight

Dispersant G-----12

Aromatic petroleum solvent (No. 40, Union Oil Company of California, or equivalent)-----18

Alkyd resin solution (50% solids in mineral spirits, No. 1323 Aroplaz, Stroock & Wittenerberg, or equivalent)-----64

The dispersant and solvent are mixed together and stirred until completely dissolved. The alkyd resin is then mixed into the mass forming a medium bodied vehicle of a clear straw color and which may be thinned with water.

## Paste paint

## Parts by weight

Titanium oxide (water dispersible preferred)-----30

Above vehicle-----25

These ingredients are thoroughly mixed together to provide a water thinnable paste paint. Thirty-five parts of water is added to reduce the paste to brush consistency. The resultant paint which is unusually white, brushes freely, hides and levels well. The dried film is smooth and free from brush marks. One coat covers excellently and after drying over night, the applied paint can be washed with cold water repeatedly.

For the next example part of the polymerized rosin is used for the dispersant and the balance is added to provide a solid combined resin and dispersant and which, of course, is not as hard as would result from a combination of polymerized rosin and a maleic resin of the type used in formula G; however, a very satisfactory product is obtained from polymerized rosin and which may be used as the sole binder with complete satisfaction for interior water thinnable paints.

## DISPERSANT H

## Parts by weight

55 Polymerized rosin (poly pale resin, Hercules Powder Company, or equivalent)-----48

Pine oil (double distilled preferred)-----1

Sodium hydroxide-----3

Borax-----1

60 Water (distilled preferred)-----8

Boiled linseed oil (pale refined preferred)-----12

Sixteen parts previously pulverized polymerized rosin, one part pine oil and four parts of water are thoroughly mixed. Three parts sodium hydroxide and one part borax are mixed together in a separate container and the remaining four parts of water are slowly added and stirred until dissolved. While the resultant solution is still hot from the heat of reaction between the alkali and water, it is immediately added to the rosin mixture and stirred a short while, less than a minute. The liquid will separate from the rosin particularly when the solids are pressed or 75 packed together and the liquid decanted. The

## 13

alkali contacted rosin is then heated until fluid, whereupon twelve parts of boiled linseed oil are slowly added with constant stirring followed with the remaining thirty-two parts of pulverized rosin and thoroughly mixed. Cooking is continued until a sample drop on glass becomes clear and brittle when cooled to room temperature, after which the mass is poured into cooling pans to harden.

This mass may be subsequently dissolved as desired by a suitable solvent to provide a water thinnable vehicle.

## EXAMPLE 7

## Vehicle

|                                                                                | Parts by weight |
|--------------------------------------------------------------------------------|-----------------|
| Dispersant H                                                                   | 50              |
| Petroleum paint thinner (No. 9 Union Oil Company of California, or equivalent) | 50              |

The above materials are mixed together in a beaker, and because of the poor solvency of the petroleum thinner, are heated on a water bath and stirred until completely dissolved. The resultant water thinnable paint vehicle has a clear light amber color.

## Paste paint

|                                              | Parts by weight |
|----------------------------------------------|-----------------|
| Titanium oxide (water dispersable preferred) | 40              |
| Above vehicle                                | 30              |

These ingredients are thoroughly mixed together to provide a water thinnable paste paint. For brush consistency, two volumes of paste paint are thinned with one volume of water. The resultant product unusually white, brushes easily, hides well and levels out into a smooth flat finish that can be readily washed with cold water after drying over night.

It will be readily apparent from a consideration of the different examples of dispersants and surface coating compositions which may be formed therewith, as set forth above, that the dispersant of the present invention is applicable throughout a broad field of surface coating compositions. Thus it is seen that both interior and exterior paints and varnishes may readily be made water thinnable. The term water thinnable is used so as to distinguish the surface coating compositions of the present invention from those which can be thinned only with water for, as stated above, the surface coating compositions prepared in accordance with the present invention may be thinned either with water or with the usual spirit thinners as desired.

Having described the invention in what are considered to be a few typical embodiments thereof it is desired that it be understood that the specific proportions and ingredients may be varied considerably without departing from the spirit and scope of the invention.

I claim:

1. The method of making a non-aqueous vehicle material for producing paint compositions capable of being thinned with water, said method comprising the steps of reacting substantially sixteen parts by weight of rosin with from one and one-half to four parts of a base selected from the group consisting of potassium and sodium hydroxide and from one-half to two and one-half parts borax, removing the liquid component of the reaction products, mixing the solid component of the reaction product with a fatty drying oil to form a heavy bodied vehicle miscible with both water and spirit thinners.

## 14

2. The process of making a composition for use as a dispersant in the production of water- and oil-thinnable coating compositions which comprises reacting about 16 parts of comminuted rosin with a mixture comprising between about 1½ and about 4 parts sodium hydroxide, between about 4 parts and about 24 parts water, between about 1 part and about 6 parts pine oil, and between about ½ part and about 2½ parts borax, wherein parts are expressed as parts by weight, the reaction being effected at a temperature of about 60° C. for a time of between about ½ minute and about 5 minutes, and separating from the resulting mixture a solid phase comprising particles of rosin having surface coatings of alkali metal rosinate.

3. The process of making a composition for use as a dispersant in the production of water-thinnable and oil-thinnable coating compositions which comprises reacting about 16 parts of a comminuted rosin with a mixture comprising between about 1½ and about 4 parts alkali metal hydroxide, between about 4 parts and about 24 parts water, between about 1 part and about 6 parts pine oil, and between about ½ part and about 2½ parts borax, parts being expressed as parts by weight, the reaction being effected at a temperature of between about 50° C. and about 100° C. for a time of between about ½ minute and about 5 minutes, and separating from the resulting mixture a solid phase comprising particles of rosin having surface coatings of alkali metal rosinate.

4. The process of making a dispersant for use in paints, varnishes and the like, which process comprises reacting about 16 parts of a comminuted rosin with about 1½ to about 4 parts alkali metal hydroxide, and about 4 parts to about 24 parts water, parts being expressed as parts by weight, at a temperature of between about 50° C. and about 100° C., for a time of between about ½ minute and about 5 minutes thereby forming a solid phase comprising alkali metal rosinate-coated rosin particles and a liquid phase comprising an aqueous solution of unreacted alkali metal hydroxide, and separating said solid phase from said liquid phase.

5. The process of making a water- and oil-thinnable dispersing composition for use in paints, varnishes and the like, which process comprises reacting about 16 parts of comminuted abietic acid, about 1½ to about 4 parts alkali metal hydroxide, and about 4 parts to about 24 parts water, parts being expressed as parts by weight, at a temperature of between about 50° C. and about 100° C. for a time of between about ½ minute and about 5 minutes thereby forming a solid phase comprising particles of abietic acid having surface coatings of alkali metal abietate and a liquid phase comprising an aqueous solution of unreacted alkali metal hydroxide, and separating said solid phase from said liquid phase.

6. The process of making a solid dispersant for coating compositions which are thinnable with aqueous and spirit thinners which process comprises reacting about 16 parts of a comminuted rosin, about 1½ to about 4 parts alkali metal hydroxide, and about 4 parts to about 24 parts water, parts being expressed as parts by weight, at a temperature of between about 50° C. and about 100° C., for a time of between about ½ minute and about 5 minutes thereby forming a solid phase comprising alkali metal rosinate-coated rosin particles and an aqueous phase containing unreacted alkali metal hydroxide, separating said

solid phase from said aqueous phase and drying said solid phase.

7. The process of making a coating composition which is thinnable with water and spirit thinners, which comprises reacting about 16 parts by weight of a comminuted rosin with an aqueous solution comprising from about 1½ parts to about 4 parts by weight of alkali metal hydroxide dissolved in from about 4 parts to about 24 parts by weight water at a temperature of from about 50° C. to about 100° C. for a reaction time of from about 0.5 minute to about 5 minutes, separating the resulting solid product comprising particles of rosin having surface coatings of alkali metal rosinate, and admixing said solid 15 product with a film-forming material.

GUSTAVUS HARRY MILLER.

## UNITED STATES PATENTS

| Number       | Name       | Date          |
|--------------|------------|---------------|
| 2,351,949    | Georgi     | June 20, 1944 |
| 1,672,377    | Exley      | June 5, 1928  |
| 2,268,112    | Dreshfield | Dec. 30, 1941 |
| 2,326,610    | Borglin    | Aug. 10, 1943 |
| 2,372,577    | Hirsch     | Mar. 27, 1945 |
| 2,116,768    | Rowland    | May 10, 1938  |
| 10 2,242,529 | Langmeier  | May 20, 1941  |
| 694,085      | Zingg      | Feb. 25, 1902 |

## FOREIGN PATENTS

| Number  | Country       | Date          |
|---------|---------------|---------------|
| 104,012 | Great Britain | Feb. 12, 1917 |

## OTHER REFERENCES

Ind. Eng. Chem., 26, 712 (1934).

## REFERENCES CITED

The following references are of record in the 20 file of this patent: